



US007455959B2

(12) **United States Patent**  
**Clark et al.**

(10) **Patent No.:** **US 7,455,959 B2**  
(45) **Date of Patent:** **Nov. 25, 2008**

(54) **PHOTOGRAPHIC ELEMENT CONTAINING A SPEED-ENHANCING COMPOUND**

(75) Inventors: **Bernard A. Clark**, Berkshire (GB); **Philip A. Allway**, Hertfordshire (GB); **Tania Zuberi**, Middlesex (GB); **Stephen P. Singer**, Spencerport, NY (US); **Charles E. Heckler**, Rochester, NY (US); **Louis E. Friedrich**, Rochester, NY (US)

(73) Assignee: **Eastman Kodak Company**, Rochester, NY (US)

(\*) Notice: Subject to any disclaimer, the term of this patent is extended or adjusted under 35 U.S.C. 154(b) by 385 days.

(21) Appl. No.: **10/574,669**

(22) PCT Filed: **Oct. 1, 2004**

(86) PCT No.: **PCT/GB2004/004184**

§ 371 (c)(1),  
(2), (4) Date: **Mar. 31, 2006**

(87) PCT Pub. No.: **WO2005/036262**

PCT Pub. Date: **Apr. 21, 2005**

(65) **Prior Publication Data**

US 2008/0248433 A1 Oct. 9, 2008

(30) **Foreign Application Priority Data**

Oct. 4, 2003 (GB) ..... 0323280.8

(51) **Int. Cl.**

**G03C 1/46** (2006.01)  
**G03C 1/06** (2006.01)  
**G03C 1/36** (2006.01)  
**G03C 1/08** (2006.01)  
**G03C 5/18** (2006.01)

(52) **U.S. Cl.** ..... **430/546**; 430/502; 430/503; 430/504; 430/505; 430/506; 430/507; 430/508; 430/509; 430/541; 430/542; 430/543; 430/599; 430/600; 430/607; 430/613; 430/614; 430/615; 430/449; 430/464; 430/401; 430/434

(58) **Field of Classification Search** ..... 430/502-509, 430/541-543, 599-600, 607, 613-615, 401, 430/434, 449, 464

See application file for complete search history.

(56) **References Cited**

**U.S. PATENT DOCUMENTS**

7,354,701 B2 \* 4/2008 Clark et al. ..... 430/502

**FOREIGN PATENT DOCUMENTS**

|    |           |         |
|----|-----------|---------|
| EP | 0 258 662 | 3/1988  |
| EP | 0 450 965 | 10/1991 |
| EP | 0 724 194 | 7/1996  |
| GB | 2 110 832 | 6/1983  |
| GB | 2 328 755 | 3/1999  |
| JP | 61-256345 | 11/1986 |

\* cited by examiner

*Primary Examiner*—Geraldina Visconti

(57) **ABSTRACT**

The invention provides a color photographic element comprising at least one light-sensitive silver halide emulsion layer or a non silver-containing light-insensitive layer, in which at least one of these layers contains a colorless imidazole compound of formula (I) that undergoes less than 10% chemical or redox reaction with oxidized developer and which enables the photographic speed of the element to be increased by at least 0.05 stop without increasing granularity, compared to the same element without the compound, wherein the compound of formula (I) has the structure:



wherein

X is H or a substituent;

Z represents the atoms necessary to complete an unsubstituted or substituted imidazole ring, which may form part of a fused unsubstituted or substituted ring system containing no further ring heteroatoms; wherein there is present at least one —NH group either in the imidazole ring or directly attached to the imidazole ring as part of X;

provided that

(a) when Z represents the atoms necessary to complete an unsubstituted or substituted benzimidazole ring, an —NH group is directly attached to the imidazole ring as part of X, and X is located between the imidazole nitrogen atoms;

(b) when the —NH group is located in the ring adjacent to the carbon atom bearing X, and X is located between the imidazole nitrogen atoms, the imidazole ring is not fused to a phenanthrene ring.

The compounds of formula (I) increase speed without a concomitant increase in size of the light-sensitive silver halide grains.

**26 Claims, No Drawings**

1

## PHOTOGRAPHIC ELEMENT CONTAINING A SPEED-ENHANCING COMPOUND

## CROSS REFERENCE TO RELATED APPLICATION

This application is cross-related to co-filed UK patent application No. 0323280.8.

## FIELD OF THE INVENTION

This invention relates to a colour photographic element containing a speed-enhancing imidazole compound in a layer containing a light-sensitive silver halide emulsion layer and/or in a non-silver containing light-insensitive layer.

## BACKGROUND OF THE INVENTION

It is a long-standing objective of origination colour photographic materials to maximize the overall response to light while maintaining the lowest possible granularity. Increased photographic sensitivity to light, commonly referred to as photographic speed, allows for improved images captured under low light conditions or improved details in the shadowed regions of the image. In general, the overall sensitivity to light provided by the light-sensitive silver halide emulsions in such systems is determined by the size of the emulsion grains. Larger emulsion grains capture more light. Upon development, the captured light is ultimately converted into dye deposits that constitute the reproduced image. However, the granularity exhibited by these dye deposits is directly proportional to the sizes of the silver halide grains. Thus, larger silver halide grains have higher sensitivity to light but also lead to higher granularity in the reproduced image. Therefore, it is a fundamental problem in photography to improve the light sensitivity of a silver halide element without a corresponding increase in granularity, hereinafter referred to as a 'speed/grain effect'. Stated from another perspective, it has been a long-standing problem to provide materials which maximise the response to light of a silver halide emulsion for any given grain size.

Many different classes of heterocyclic materials are known to affect silver development in some manner and have been called, for example, antifoggants, fog restrainers, development restrainers, development inhibitors and stabilizers. Descriptions of these materials can be found in *The Fundamentals of Photographic Technology, Silver Salt Photography*, compiled by the Photographic Society of Japan (Corona, Ltd.), p 354; *Chemistry of Photography*, A. Sasai (Shashin Kogyo Shuppan Co, Ltd.), pp 168-169 and T. H. James, Ed, *The Theory of the Photographic Process*, 4<sup>th</sup> Edition, Macmillan Publishing Co, NY, Chapter 13, Section J. Commonly, these materials all contain an —NH or —SH group which allows them to bond or strongly adsorb to the silver surface and whose silver salts have a  $pK_{sp}$  ( $-\log K_{sp}$ ) of more than 10, wherein  $K_{sp}$  is the solubility product in water at 25C.

It is well known to add these materials to silver halide emulsions in conventional colour photographic systems to limit or decrease their development. These materials are generally at least partially water-soluble or soluble in water-miscible solvents such as methanol and are added directly to silver emulsions before coating of the film or added directly to the developer solutions. It is also known to attach these types of heterocycles covalently to PUGs (photographically useful groups) so that the PUG will be held in close proximity to the silver surface see, for example, in U.S. Pat. No. 5,100,761.

2

U.S. Pat. Nos. 5,032,499, U.S. Pat. No. 4,837,141 and JP 62-138850 describe the use of a wide variety of photographic restrainers, including diazoles, in thermally developable light-sensitive materials. JP 10-50047 describes a wide variety of anti-silver sludging agents, including diazoles, in a non-light-sensitive cleaning film and JP 63-24255 describes a wide variety of diazoles in a colour photographic film.

US Patent Application Publication No. 2002/0045138 discloses certain imidazoles that can be used in photographic materials to improve granularity without an increase in fogging. The imidazoles are required to be N-substituted unless two adjacent substituents join to form a phenanthrene ring.

U.S. Pat. No. 5,187,054 discloses a photographic material which comprises a ballasted heterocycle, such as a benzimidazole, located in a non light-sensitive layer to reduce sludge formed during the development process but these compounds do not give a 'speed/grain effect'.

U.S. Pat. No. 5,702,877 describes the use of ballasted benzimidazoles to improve granularity with certain pyrazolone image couplers.

U.S. Pat. No. 6,319,660 describes speed-improving compounds with, specifically, at least three heteroatoms in the ring system in a layer that contains a light-sensitive silver halide emulsion or in a non silver-containing light-insensitive layer. Among the speed-improving compounds described are purines, benzotriazoles, triazoles and thiadiazoles. Indeed generally it had been considered that for a 'speed/grain' effect to be observed, it was necessary for a heterocyclic compound to have at least three heteroatoms in the ring system, thereby limiting the range of suitable compounds.

## PROBLEM TO BE SOLVED BY THE INVENTION

It is highly desirable to extend the range of compounds that can provide an imaging material with increased photographic speed without increase in the size of the light-sensitive silver halide grains, or that can provide the same photographic speed with smaller light-sensitive silver halide gains, especially if those compounds can be synthesized more economically and/or are more readily available.

## SUMMARY OF THE INVENTION

According to the present invention there is provided a colour photographic element comprising at least one light-sensitive silver halide emulsion layer or a non silver-containing light-insensitive layer, in which at least one of these layers contains a colourless imidazole compound of formula (I), that undergoes less than 10% chemical or redox reaction directly with oxidized developer and which enables the photographic speed of the element to be increased by at least 0.05 stop without increasing granularity, compared to the same element without the compound, wherein the compound of formula (I) has the structure:



wherein

X is H or a substituent;

Z represents the atoms necessary to complete an unsubstituted or substituted imidazole ring, which may form part of a fused unsubstituted or substituted ring system containing no further ring heteroatoms;

wherein there is present at least one —NH group either in the imidazole ring or directly attached to the imidazole ring as part of X;

provided that

(a) when Z represents the atoms necessary to complete an unsubstituted or substituted benzimidazole ring, an —NH group is directly attached to the imidazole ring as part of X, and X is located between the imidazole nitrogen atoms;

(b) when the —NH group is located in the ring adjacent to the carbon atom bearing X, and X is located between the imidazole nitrogen atoms, the imidazole ring is not fused to a phenanthrene ring.

In another embodiment of the invention there is provided a multi-colour photographic element comprising a support bearing yellow, magenta and cyan image-dye-forming units comprising at least one blue-, green- or red-sensitive silver halide emulsion layer having associated therewith at least one yellow, magenta or cyan dye-forming coupler respectively, wherein the element is as herein described.

In yet another embodiment of the invention there is provided a process of forming an image in a photographic element as hereinbefore defined after the element has been imagewise exposed to light, comprising contacting the element, as herein described, with a colour developing agent.

#### ADVANTAGEOUS EFFECT OF THE INVENTION

The imidazole compounds for use in the invention increase speed without a concomitant increase in size of the light-sensitive silver halide grains and hence the granularity, increasing the range of compounds that exhibit this 'speed/grain effect'. They are generally easier to synthesise and/or more readily available than their counterparts having at least three heteroatoms in the ring system.

#### DETAILED DESCRIPTION OF THE INVENTION

The invention is generally as described in the Summary of the Invention. The imidazole compounds are colourless, so that excluded from the scope are coloured materials or dyes such as, for example, sensitizing dyes, filter dyes and anti-halation dyes.

The phrase that the imidazole compound "undergoes less than 10% chemical or redox reaction directly with oxidized developer" is meant to be an in-film result following the development step(s) of the photographic process. This restriction is made to distinguish such a compound from other photographic materials that are commonly known to react to a greater extent with oxidized developer, such as but not limited to, couplers, scavengers of oxidized developer and electron transfer agents. This can be tested by standard analysis of a standard film before and after standard processing for the presence of the compound, wherein any loss of imidazole compound caused by the processing should be less than 10% conversion in the compound.

Thus the imidazole compounds for use in the invention are not couplers and do not react with oxidized developer ( $D_{ox}$ ) to generate dyes or any other product by undergoing any significant amounts (less than 10%, preferably less than 5%) of chemical or redox reaction directly with oxidized colour developer. They should be stable to other components of the processing solutions and not contain substituents that undergo substantial amounts of chemical reaction in any of

the processing solutions. For example, the imidazole compounds may not contain hydrazino or hydroquinone groups that may cross-oxidize during silver development, nor may they be covalently linked to any other kind of photographic useful group (PUG). However, they may contain, for example, ester substituents that are not substantially hydrolyzed (less than 5-10%) during the development process.

The imidazole compounds for use in the invention achieve an improvement in terms of photographic speed of at least 0.03, desirably at least 0.05, more desirably at least 0.10 and even 0.25 stops or more, compared to the coating without the compound, without causing a significant increase in granularity.

By one-stop increase in speed is meant that 50% of the standard amount of scene light gives the same photographic effect as a coating that does not have such a speed increase. The formula that relates 'stop' to light exposure is

$$\log(E/E_s) = (\text{stop})\log(0.50),$$

wherein stop is the measure of speed increase,  $E_s$  is the standard exposure, and  $E/E_s$  is the fractional exposure required as a result of the increase in speed. For example, a zero-stop increase means  $E/E_s$  is unity. A 1-stop increase in speed means  $E/E_s$  is 0.50. A 0.10-stop increase in speed corresponds to an  $E/E_s$  equal to 0.93. A 0.03 stop increase in speed corresponds to an  $E/E_s$  equal to 0.98.

These compounds are located in the film element as described and are not added to the processing solutions.

Included within the scope of this invention are polycyclic imidazole compounds, preferably having from 5 to 9 carbon atoms in the fused ring, provided there are no further ring heteroatoms in that ring, such as, for example, a benzimidazole.

Typically a satisfactory speed increase is found when the imidazole compound is substituted with groups that together contain at least eight, preferably at least twelve, more preferably at least fourteen, carbon atoms.

As used herein and throughout the specification unless where specifically stated otherwise, the term "alkyl" refers to an unsaturated or saturated, straight or branched chain alkyl group, including alkenyl and aralkyl, and includes cyclic alkyl groups, including cycloalkenyl, having 3-8 carbon atoms and the term "aryl" includes specifically fused aryl.

The term "heteroatom" as used herein encompasses any atom other than carbon or hydrogen and includes, for example, nitrogen, sulfur, phosphorous and oxygen.

Any substituents located directly on the heterocycles useful in the invention may be chosen such that together the entire compound meets an overall partition coefficient requirement. They may be, for example, halo, such as fluoro, chloro, bromo or iodo, cyano, hydroxy, nitro or unsubstituted or substituted alkyl, aryl, alkoxy or aryloxy, alkyl- or aryl-thio, mercapto, alkyl- or aryl-sulfinyl, alkyl- or aryl-sulfonyl, alkyl- or aryl-acylamino, alkyl- or aryl-ureido, alkyl- or aryl-carbamato, alkyl- or aryl-sulfonylamino, alkyl- or aryl-sulfamoyl, alkyl- or aryl-oxycarbonyl, alkyl- or aryl-oxysulfonyl, a heterocyclic group, such as furanyl or morpholino, a carbonyl group, such as keto, formyl, carboxylic acid, alkyl- or aryl-carbonyl, alkyl- or aryl-carbamoyl, alkyl- or aryl-carbonamido or an alkyl- or aryl-amino group, such as a primary, secondary or tertiary substituted nitrogen. These groups may be further substituted, for example with one or more of the above groups, which may in turn be further substituted. In addition, the substituent may further contain a group that can be incorporated into a polymeric backbone. It should be noted

5

that alternative tautomeric structures of the imidazole nucleus are considered to be chemically equivalent and are part of the invention.

It has been found that in most cases in order to show the optimum 'speed/grain effect' the imidazole compound of formula (I) will have one or more electron-withdrawing groups attached to the imidazole ring, to a ring fused thereto or as part of substituent X.

By electron-withdrawing group is meant a group with a positive Hammett  $\sigma$  value, as described by Hansch et al in Chem. Rev. 1991 91 165-195 'A Survey of Hydrogen Substituent Constants and Resonance Field Parameters'. Suitable groups may include, for example, a cyano, carbonyl, alkoxy-carbonyl, trifluoromethyl, sulfonyl, sulfoxyl or thio group.

When there is an —NH group in the imidazole ring, X may be, for example, a cyano or an unsubstituted or substituted alkyl, aryl, alkyl- or aryl-sulfonyl, alkyl- or aryl-carbonyl, alkyloxy- or aryloxy-carbonyl or heterocycl group such as, for example, furanyl, or a group NRQR<sup>1</sup>, wherein R is hydrogen or an alkyl group, more preferably hydrogen, R<sup>1</sup> is a substituent and Q is, in particular, a carbonyl, sulfonyl or aryl group.

However preferably there is an —NH group directly attached to the imidazole ring as part of X. Thus, in a more preferred embodiment, the general structure of the speed-enhancing compound corresponds to formula (II):—



wherein

NHQ is selected from the class consisting of amido, arylamino, ureido, carbamato or sulfonamido;

R<sup>1</sup> is a substituent; and

*Z* represents the atoms necessary to complete an unsubstituted or substituted imidazole ring, which may form part of a fused unsubstituted or substituted ring system containing no further ring heteroatoms;

provided that when Z represents the atoms necessary to complete an unsubstituted or substituted benzimidazole ring, NHQR<sup>1</sup> is located between the two imidazole nitrogen atoms.

Typically, for example Q is or contains an electron-withdrawing group, such as a carbonyl group or a sulfonyl group, such that the group NHQ is an amido, ureido, carbamato or sulfonamido group. When NHQ is an amido or ureido group generally it will be found to be advantageous for there to be present one or more further electron-withdrawing groups on the heterocyclic ring or ring system. When NHQ is a sulfonamido group, then the ring or ring system may be unsubstituted or substituted with one or more electron-withdrawing or electron-donating groups. For those compounds wherein Q is not an electron-withdrawing group, for example an aryl group, then generally it has been found that one or more electron-withdrawing groups will be required on the heterocyclic ring or ring system.

6

More particularly the imidazole will have a structure (III):—



wherein

$R^1, R^2, R^3$  and  $R^4$  are independently selected substituents or  $R^3$  and  $R^4$  may join to form a ring not containing any ring heteroatoms;

NHQ is selected from the class consisting of an amido, ureido arylamino, carbamato or sulfonamido group.

Preferably  $R^1$  is selected from hydrogen and an unsubstituted or substituted alkyl, aryl, alkoxy, aryloxy, or alkyl- or aryl-amino group. When Q is or contains a carbonyl group then  $R^1$  is preferably an alkyl group which is unsubstituted or substituted, for example, with an aryloxy group, which may itself be substituted, for example with one or more alkyl groups. When Q is or contains a sulfonyl group,  $R^1$  is preferably an aryl group, in particular substituted with an alkyl carbonamido group, which may itself be substituted. When Q is an aryl group then  $R^1$  may, for example, be an alkoxy group.

Preferably Q is a carbonyl or sulfonyl group and R<sup>2</sup> is hydrogen or an unsubstituted or substituted alkyl group. More preferably, at least one of R<sup>3</sup> and R<sup>4</sup> is hydrogen or a group which is independently selected, for example, from cyan, formyl, keto, carboxylic acid, mercapto and unsubstituted or substituted alkyl (including specifically trifluoromethyl), aryl, alkoxy, aryloxy, alkoxy- or aryloxy-carbonyl, alkyl- or aryl-carbonyl, alkyl- or aryl-thio, alkyl- or aryl-sulfoxyl, alkyl- or aryl-sulfonyl, alkyl- or aryl-carbamoyl and alkyl- or aryl-carbonamido, which may be further substituted with one or more such groups, or R<sup>3</sup> and R<sup>4</sup> may join to form a fused ring, for example a phenyl ring, which may be substituted.

The following are examples of imidazole compounds that are useful in this invention:



-continued



SGA5 15



SGA6 25



SGA7



SGA8 40



SGA9 50



SGA10



60

65

-continued



SGA12 15



SGA13 25



SGA14 30



SGA15 35



SGA16 40



SGA17





-continued

For each compound useful in the invention, as the laydown is increased a threshold level is reached following which the speed improvement gradually increases with laydown, after which the improvement then levels off at a compound specific maximum level. It will be appreciated that the amount is also a function of other variables such as the location and number of layers in which the compound is located, the solvent used and film dimensions. Thus, it is desirable to have enough laydown of the compound in order to obtain the speed improvement. Sufficient laydown is required to achieve an improvement of at least 0.03, desirably 0.05 and more desirably at least 0.10 and even 0.25 stops or more.

Where the imidazole compound is present in a sensitized layer, the ratio of compound to silver is suitably at least 0.1 mmol of compound per mol of silver halide and, more pref-

## 11

erably, at least 1.0 mmol of compound per mol of silver halide and, most preferably, at least 2.0 mmol per mol of silver halide. When coated in a non-silver-containing layer, the laydown of the compound is suitably at least  $3 \times 10^{-5}$  mol/m<sup>2</sup>, more preferably at least 0.0001 mol/m<sup>2</sup>.

The materials useful in the invention can be added to a mixture containing silver halide before coating or be mixed with the silver halide just prior to or during coating. In either case, additional components like couplers, doctors, surfactants, hardeners and other materials that are typically present in such solutions may also be present at the same time.

The materials useful in the invention are not water-soluble and cannot be added directly to the solution. They may be added directly if dissolved in an organic water-miscible solvent such as, for example, methanol or acetone or more preferably as a dispersion. A dispersion incorporates the material in a stable, finely divided state in a lipophilic organic solvent (often referred to as a permanent solvent) that is stabilized by suitable surfactants and surface-active agents, usually in combination with a binder or matrix such as gelatin. The dispersion may contain one or more permanent solvents that dissolve the material and maintain it in a liquid state.

Some examples of suitable permanent solvents are tricresylphosphate, N,N-diethylauramide, N,N-dibutylauramide, p-dodecyl-phenol, dibutylphthalate, di-n-butyl sebacate, N-n-butylacetanilide, 9-octadecen-1-ol, ortho-methylphenyl benzoate, trioctylamine and 2-ethylhexylphosphate. Permanent solvents can also be described in terms of physical constants such as alpha, beta and pi\* as defined by M. J. Kamlet, J-L. M. Abboud, M. H. Abraham and R. W. Taft, *J. Org Chem*, 48, 2877 (1983). The preferred permanent solvents used with the materials useful in the invention are those with Log Kow of 5.0 or greater and beta values of 0.4 or greater, more preferably 0.5 or greater.

Preferred classes of solvents are carbonamides, phosphates, alcohols and esters. When a solvent is present, it is preferred that the weight proportion of compound to solvent be 1 to at least 0.5, more preferably 1 to at least 1.

The partition coefficient of a compound provides a means of gauging its lipophilicity but this is not a convenient property to measure. Because it can be difficult to measure logP values above 3, a model can be used to compute an estimate of logP that defines the limits of the invention.

ClogP can be used as a predictor of logP and the model used in U.S. Pat. No. 6,319,660 utilizes the software program by W. Meylan from Syracuse Research Corporation, 6225 Running Ridge Road, North Syracuse, N.Y., 13212. The compound whose logP is desired is entered into the program called KowWin, 32-bit Version 1.66, written in year 2000. The computed logP is then called Log Kow. A literature article that describes the program is W. M. Meylan and P. H. Howard, 'Atom/fragment contribution method for estimating octanol-water partition coefficients', *J. Pharm. Sci.* 84: 83-92, 1995.

The dispersion may require an auxiliary coupler solvent initially to dissolve the component but this is removed afterwards, usually either by evaporation or by washing with additional water. Some examples of suitable auxiliary coupler solvents are ethyl acetate, cyclohexanone and 2-(2-butoxyethoxy)ethyl acetate. The dispersion may also be stabilized by addition of polymeric materials to form stable latexes. Examples of suitable polymers for this use generally contain water-solubilizing groups or have regions of high lipophobicity. Some examples of suitable dispersing agents or surfactants are Alkanol XC™ or saponin. The materials useful in the invention may also be dispersed in admixture with another component of the system, such as a coupler or an oxidized developer scavenger, so that both are present in the same oil

## 12

droplet. It is also possible to incorporate the materials useful in the invention as a solid particle dispersion; i.e. as a slurry or suspension of finely, mechanically ground compound. Such a solid particle dispersion may be additionally stabilized with surfactants and/or polymeric materials as known in the art. Also, additional permanent solvent may be added to the solid particle dispersion to help increase activity.

The sensitivity of the human eye is greatest to green light and so the imidazole compounds are most useful when located in the green record (the layer whose maximum spectral sensitivity to light is from 500 to 600 nm).

The following magenta couplers are particularly beneficial when used in conjunction with the imidazole compounds useful in the invention:

15

M-1:



20

30

M-2:



35

M-3:



45

M-4:



55

60

65

**13**

-continued

M-5:



M-6:



M-7:



M-8:

**14**

-continued

M-9:



M-10:



M-11:



**15**

M-12:

-continued

**16**

The following green sensitizing dyes are also particularly beneficial when used in combination with the imidazole compounds useful in the invention:—



M-11:



M-12:



-continued

GSD-3:



GSD-4:



GSD-5:



GSD-6:



GSD-7:



GSD-8:



GSD-9:



-continued

GSD-10:



The imidazole compounds are also useful when located in the red record (the layer whose maximum spectral sensitivity to light is from 600 and 700 nm). The following cyan couplers

are particularly beneficial when used in conjunction with these imidazole compounds.



-continued

C-6



C-7



C-8



C-9



C-10



The following red sensitizing dyes are also particularly beneficial when used in combination with the imidazole compounds useful in the invention:—

RSD-4:



RSD-5:



RSD-6:



RSD-7:



The type of light-sensitive silver halide emulsion used in the layer that contains the imidazole compound may be important to obtain the desired increase in light sensitivity. The silver halide emulsion is suitably a silver iodobromide emulsion, that is an emulsion that is low in chloride. By low in chloride, it is meant that there should be present in the layer

no more than 20 mol % chloride, more suitably no more than 10 mol % chloride, typically no more than 1 mol % chloride. The silver halide grains comprise at least 50, preferably 70 and optimally at least 90 mol % bromide based on silver and at least 0.01, preferably 0.5 and optimally at least 1.0 mol % iodide based on silver, with any remaining halide being chloride. Additional iodide may be incorporated to serve other functions, such as increased native blue absorption or inter-image effects.

10 The benefit of the increase in light sensitivity is most apparent in combination with larger-sized emulsions that are associated with increased granularity. Thus, it is preferred that the compounds useful in the invention are used with emulsions that have an equivalent circular diameter of at least 0.6  $\mu\text{m}$ , or more preferably at least 0.8  $\mu\text{m}$ , or most preferably at least 1.0  $\mu\text{m}$ . In addition, the benefit of the invention is greatest in origination materials such as colour negative or colour reversal materials, since they require higher sensitivity to light 15 (because of the variable lighting conditions in natural scenes) and low granularity (due to high magnification), relative to colour print materials for which exposure conditions are carefully controlled and which are viewed directly under low magnification conditions.

20 25 The imidazole compounds are also particularly useful when used in film elements that contain low overall silver levels. Thus, films containing 9  $\text{g}/\text{m}^2$  of total silver or less, or more preferably 5.4  $\text{g}/\text{m}^2$  or less or even 4.3  $\text{g}/\text{m}^2$  or less benefit from the use of such compounds.

30 35 In order to control and maintain granularity over a wide exposure range, it is a common practice to divide an individual colour record into separate layers, each containing silver halide emulsions of different degree of sensitivity to the same colour of light. While the compound for use in the invention is most useful in the most light-sensitive layer, it can be used in more than one record that is sensitive to the same colour of light to provide greater latitude of the film to large 40 ranges of scene exposure. When two or more such sublayers exist, the most light-sensitive layer is the sublayer that responds to the lowest levels of scene exposure, unlike the other sublayers that require greater scene exposures.

45 For example, in a colour record, such as the green record, that is split into three layers of different relative sensitivity; fast (F), mid (M) or slow (S), the compound can be used in each layer only, or in any combination; i.e., for example, F+M, F+M+S and F+S. It is not necessary that these layers be adjacent, i.e. they may have interlayers or even imaging layers that are sensitive to other colours located between them. In addition, although the most light-sensitive layer is typically 50 located in the film structure closest to the exposure source and farthest from the support, the compounds useful in the invention allow for alternative locations of the layers. For example, 55 a more light-sensitive layer containing the compound useful in the invention may be located below (farther from the exposing source) than a less sensitive layer.

60 The preferred layer in which the compounds useful in the invention are used is the light-sensitive layer that is the most light-sensitive of two or more light-sensitive layers having the same spectral sensitivity. It is especially preferred that the most light-sensitive layer uses a silver iodobromide emulsion.

65 It is also possible to use the compounds useful in the invention in more than one colour record at a time. Moreover, when a number of layers of the same spectral sensitivity but of differing degrees of sensitivity to light are used, it is known

25

that overall granularity can be minimized by using a smaller molar amount of dye-forming coupler than silver in the layers of higher sensitivity. Thus, it is preferred that the layers containing the compound useful in the invention additionally contain less than a stoichiometric amount of total dye forming coupler(s) relative to the amount of silver contained in the same layer. A suitable molar ratio of dye-forming coupler(s) to silver in the layer containing the compound useful in the invention would be less than 0.5, preferably 0.2 or even 0.1 or less.

It is known that film elements that contain silver halide emulsions in one layer that have maximum sensitivities that are separated or shifted from emulsions in other layers that are sensitive to the same colour of light are useful for increasing the amount of interimage and improving colour reproduction. For example, a layer containing an emulsion may have maximum sensitivity at ~530 nm, whereas another layer contains a different green light-sensitive emulsion may be most sensitive at ~550 nm. The layer containing the emulsions with shifted sensitivities may not contain any image couplers at all, but rather only inhibitor-releasing couplers (DIRs or DLARs (Development Inhibitor Anchiomeric Releasing couplers)) or coloured masking couplers. The imidazole compounds are particularly useful therein since they allow for the improved colour reproduction while maintaining or increasing speed of the element.

The imidazole compounds do not tend to increase the  $D_{min}$  of the emulsion layer in which they are coated. Nevertheless, it is advantageous to use such compounds in combination with any of the antifoggants or scavengers known in the art to be useful in controlling  $D_{min}$  or fog. Specific examples of scavengers for oxidized developers would be 2,5-di-t-octylhydroquinone, 2-(3,5-bis(2-hexyldodecylamido)benzimidodo)-1,4-hydroquinone, 2,4-(4-dodecyloxybenzenesulfonamido)phenol, 2,5-dihydroxy-4-(1-methylheptadecyl)benzenesulfonic acid or 2,5-di-s-dodecylhydroquinone. Specific examples of useful antifoggants are compounds AF-1 to AF-8 whose structures are shown below, as well as 4-hydroxy-6-methyl-1,3,3a,7-tetraazaindene:

AF-1:



AF-2:



26

-continued

AF-3:



5

AF-4:



10

AF-5:



15

AF-6:



20

AF-7:



25

AF-8:



40

AF-9:

45

AF-10:

50

The hydrogen in the group —NH, present on the imidazole compound, may be optionally replaced with a group that is removed in a non-imagewise fashion during the development step to regenerate the original —NH group. Any of the temporary blocking groups known in the art to decompose in the developer in a non-imagewise manner can be used for this purpose. Particularly useful are those blocking groups that rely on some specific component of the developer solution to cause decomposition and regeneration of the original substituent. One example of this kind of blocking group that relies on the hydroxylamine present in the developer is described in U.S. Pat. No. 5,019,492.

Unless otherwise specifically stated or when the term "group" is used, it is intended throughout this specification, when a substituent group contains a substitutable hydrogen, it

is intended to encompass not only the substituent's unsubstituted form, but also its form further substituted with any group or groups as herein mentioned, so long as the group does not destroy properties necessary for photographic utility. Suitably, a substituent group may be bonded to the remainder of the molecule by an atom of carbon, silicon, oxygen, nitrogen, phosphorous or sulfur. The substituent may be, for example halo such as chloro, bromo, iodo or fluoro; nitro; hydroxy; cyano; carboxyl; or groups which may be further substituted, such as alkyl, including straight or branched chain or cyclic alkyl, such as methyl, trifluoromethyl, ethyl, t-butyl, 3-(2,4-di-t-pentyl-phenoxy)propyl and tetradecyl; alkenyl, such as vinyl and 2-butene; alkoxy, such as methoxy, ethoxy, propoxy, butoxy, 2-methoxyethoxy, sec-butoxy, hexyloxy, 2-ethylhexyloxy, tetradecyloxy, 2-(2,4-di-t-pentylphenoxy)ethoxy and 2-dodecyl-oxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy and p-tolylxy; carboxamido, such as acetamido, benzamido, butyramido, tetradecanamido, alpha-(2,4-di-t-pentylphenoxy)acetamido, alpha-(2,4-di-t-pentylphenoxy)butyramido, alpha-(3-pentadecylphenoxy)hexanamido, alpha-(4-hydroxy-3-t-butylphenoxy)tetradecanamido, 2-oxo-1-pyrrolidinyl, 2-oxo-5-tetradecyl-1-pyrrolinyl, N-methyltetradecanamido, succinimido, phthalimido, 2,5-dioxo-1-oxazolidinyl, 3-dodecyl-2,5-dioxo-1-imidazolyl and N-acetyl-N-dodecylamino, ethoxycarbonylamino, phenoxy carbonylamino, benzyloxy carbonylamino, hexadecyloxy carbonylamino, 2,4-di-t-butylphenoxy carbonyl-amino, phenyl carbonylamino, 2,5-(di-t-pentylphenyl)carbonylamino, p-dodecylphenyl carbonylamino, p-tolyl carbonylamino, N'-methylureido, N',N'-dimethyl-ureido, N'-methyl-N'-dodecylureido, N'-hexadecylureido, N',N'-dioctadecyl-ureido, N',N'-diethyl-N-ethylureido, N'-phenylureido, N',N'-diphenylureido, N'-phenyl-N'-p-tolylureido, N'-(m-hexadecylphenyl)ureido, N',N'-(2,5-di-t-pentylphenyl)-N-ethylureido and t-butylcarboxamido; sulfonamido, such as methanesulfonamido, benzenesulfonamido, p-toluenesulfonamido, p-dodecyl-benzenesulfonamido, N-methyltetradecanesulfonamido, N',N'-dipropylsulfamoyl-amino and hexadecanesulfonamido; sulfamoyl, such as N-methylsulfamoyl, N-ethylsulfamoyl, N,N-dipropylsulfamoyl, N-hexadecylsulfamoyl, N,N-dimethyl-sulfamoyl, N-[3-(dodecyloxy)propyl]sulfamoyl, N-[4-(2,4-di-t-pentylphenoxy)-butyl]sulfamoyl, N-methyl-N-tetradecylsulfamoyl and N-dodecylsulfamoyl; carbamoyl, such as N-methylcarbamoyl, N,N-dibutylcarbamoyl, N-octadecyl-carbamoyl, N-[4-(2,4-di-t-pentylphenoxy)butyl]carbamoyl, N-methyl-N-tetra-decylcarbamoyl and N,N-diethylcarbamoyl; acyl, such as acetyl, (2,4-di-t-amyl-phenoxy)acetyl, phenoxy carbonyl, p-dodecyloxyphenoxycarbonyl, methoxy-carbonyl, butoxy-carbonyl, tetradecyloxy carbonyl, ethoxycarbonyl, benzyloxy-carbonyl, 3-pentadecyloxy carbonyl and dodecyloxy carbonyl; sulfonyl, such as methoxysulfonyl, octyloxysulfonyl, tetradecyloxysulfonyl, 2-ethylhexyloxy sulfonyl, phenoxy sulfonyl, 2,4-di-t-pentylphenoxy sulfonyl, methylsulfonyl, octylsulfonyl, 2-ethylhexylsulfonyl, dodecylsulfonyl, hexadecylsulfonyl, phenylsulfonyl, 4-nonylphenylsulfonyl and p-tolylsulfonyl; sulfonyloxy, such as dodecylsulfonyloxy and hexadecylsulfonyloxy; sulfinyl, such as methylsulfinyl, octylsulfinyl, 2-ethylhexylsulfinyl, dodecylsulfinyl, hexadecylsulfinyl, phenyl-sulfinyl, 4-nonylphenylsulfinyl and p-tolylsulfinyl; thio, such as ethylthio, octylthio, benzylthio, tetradecylthio, 2-(2,4-di-t-pentylphenoxy)ethylthio, phenylthio, 2-butoxy-5-t-octylphenylthio and p-tolylthio; acyloxy, such as acetoxy, benzoyloxy, octade-

canoyloxy, p-dodecylamidobenzoyloxy, N-phenyl-carbamoyloxy, N-ethylcarbamoyloxy and cyclohexylcarbonyloxy; amino, such as phenylamino, 2-chlorophenylamino, diethylamino and dodecylamino; imido, such as N-(propanoyl)benzamido, succinimido and 3-benzylhydantoinyl; phosphato, such as dimethylphosphato and ethylbutylphosphato; phosphono, such as diethyl and dihexylphosphono; a heterocyclic group, a heterocyclic oxy group or a heterocyclic thio group, each of which may be substituted and which contain a 10 3- to 7-membered heterocyclic ring composed of carbon atoms and at least one hetero atom selected from the group comprising oxygen, nitrogen and sulfur, such as 2-furyl, 2-thienyl, 2-benzimidazolyloxy or 2-benzothiazolyl; quaternary ammonio such as triethylammonio; and silyloxy, such as trimethylsilyloxy.

If desired, the substituents may themselves be further substituted one or more times with the described substituent groups. The particular substituents used may be selected by those skilled in the art to attain the desired photographic properties for a specific application and can include, for example, lipophilic groups, solubilizing groups, blocking groups, releasing or releasable groups. Generally, the above groups and substituents thereof may include those having up to 48 carbon atoms, typically 1 to 36 carbon atoms and usually less than 24 carbon atoms, but greater numbers are possible depending on the particular substituents selected.

To control the migration of various components, it may be desirable to include a high molecular weight or polymeric backbone containing lipophilic or "ballast" group in molecules. Representative ballast groups include substituted or unsubstituted alkyl or aryl groups containing 8 to 48 carbon atoms. Representative substituents on such groups include alkyl, aryl, alkoxy, aryloxy, alkylthio, hydroxy, halo, alkoxy-carbonyl, aryloxycarbonyl, carboxy, acyl, acyloxy, amino, anilino, carboxamido, carbamoyl, alkylsulfonyl, arylsulfonyl, sulfonamido and sulfamoyl groups, wherein the substituents typically contain 1 to 42 carbon atoms. Such substituents can also be further substituted.

As used herein, the term "colour photographic element" means any element containing a light-sensitive silver halide emulsion layer containing an image dye-forming coupler. They can be single colour elements or multicolour elements. Multicolour elements contain image dye-forming units sensitive to each of the three primary regions of the spectrum. 45 Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer. A single colour element may comprise a combination of couplers in one or more common layers which upon processing together form a monocolour, including black or gray, (so-called chromogenic black and white) dye image.

A typical colour photographic element comprises a support bearing a cyan dye image-forming unit comprising at least one red-sensitive silver halide emulsion layer having associated therewith at least one cyan dye-forming coupler, a 60 magenta dye image-forming unit comprising at least one green-sensitive silver halide emulsion layer having associated therewith at least one magenta dye-foaming coupler and a yellow dye image-forming unit comprising at least one blue-sensitive silver halide emulsion layer having associated therewith at least one yellow dye-forming coupler. The element can contain additional layers, such as filter layers, inter-layers, overcoat layers or subbing layers.

If desired, the photographic element can be used in conjunction with an applied magnetic layer as described in *Research Disclosure*, November 1992, Item 34390 published by Kenneth Mason Publications, Ltd., Dudley Annex, 12a North Street, Emsworth, Hampshire PO10 7DQ, ENGLAND and as described in Hatsumi Kyoukai Koukai Gihou No. 94-6023, published Mar. 15, 1994, available from the Japanese Patent Office, the contents of which are incorporated herein by reference. When it is desired to employ the inventive materials in a small format film, *Research Disclosure*, June 1994, Item 36230 provides suitable embodiments.

In the following discussion of suitable materials for use in the emulsions and elements of this invention, reference will be made to *Research Disclosure*, September 1996, Item 38957, available as described above, which is referred to herein by the term "Research Disclosure". The contents of the *Research Disclosure*, including the patents and publications referenced therein, are incorporated herein by reference, and the Sections hereafter referred to are Sections of the *Research Disclosure*.

Except as provided, the silver halide emulsion containing elements employed in this invention can be either negative-working or positive-working, as indicated by the type of processing instructions (i.e. colour negative, reversal or direct positive processing) provided with the element. Suitable emulsions and their preparation as well as methods of chemical and spectral sensitization are described in Sections I through V of *Research Disclosure*. Various additives such as UV dyes, brighteners, antifoggants, stabilizers, light absorbing and scattering materials and physical property modifying addenda such as hardeners, coating aids, plasticizers, lubricants and matting agents are described, for example, in Sections II and VI through VIII. Colour materials are described in Sections X through XIII. Suitable methods for incorporating couplers and dyes, including dispersions in organic solvents, are described in Section X(E). Scan facilitating is described in Section XIV. Supports, exposure, development systems, and processing methods and agents are described in Sections XV to XX.

The information contained in the September 1994 *Research Disclosure*, Item No. 36544, is updated in the September 1996 *Research Disclosure*, Item No. 38957. Certain desirable photographic elements and processing steps, including those useful in conjunction with colour reflective prints, are described in *Research Disclosure*, Item 37038, February 1995.

Coupling-off groups are well known in the art. Such groups can determine the chemical equivalency of a coupler, i.e., whether it is a 2-equivalent or a 4-equivalent coupler, or modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation or colour correction.

The presence of hydrogen at the coupling site provides a 4-equivalent coupler, and the presence of another coupling-off group usually provides a 2-equivalent coupler. Representative classes of such coupling-off groups include, for example, chloro, alkoxy, aryloxy, heterooxy, sulfonyloxy, acyloxy, heterocyclol, benzotriazolyl, sulfonamido, tetrazolylthio, benzothiazolyl-thio, 2-carboxyethylthio, phosphonyloxy, arylthio and arylidiazenyl. These coupling-off groups are described in the art, for example, in U.S. Pat. Nos. 2,455,169, 3,227,551, 3,432,521, 3,476,563, 3,617,291, 3,880,661, 4,052,212 and 4,134,766; and in UK. Patents and published

application Nos. 1,466,728, 1,531,927, 1,533,039, 2,006,755A and 2,017,704A, the disclosures of which are incorporated herein by reference.

Image dye-forming couplers may be included in the element such as couplers that form cyan dyes upon reaction with oxidized colour developing agents that are described in such representative patents and publications as: "Farbkuppler-eine Literaturübersicht," published in Agfa Mitteilungen, Band III, pp. 156-175 (1961) as well as in U.S. Pat. Nos. 2,367,531; 2,423,730; 2,474,293; 2,772,162; 2,895,826; 3,002,836; 3,034,892; 3,041,236; 4,333,999; 4,746,602; 4,753,871; 4,770,988; 4,775,616; 4,818,667; 4,818,672; 4,822,729; 4,839,267; 4,840,883; 4,849,328; 4,865,961; 4,873,183; 4,883,746; 4,900,656; 4,904,575; 4,916,051; 4,921,783; 4,923,791; 4,950,585; 4,971,898; 4,990,436; 4,996,139; 5,008,180; 5,015,565; 5,011,765; 5,011,766; 5,017,467; 5,045,442; 5,051,347; 5,061,613; 5,071,737; 5,075,207; 5,091,297; 5,094,938; 5,104,783; 5,178,993; 5,813,729; 5,187,057; 5,192,651; 5,200,305; 5,202,224; 5,206,130; 5,208,141; 5,210,011; 5,215,871; 5,223,386; 5,227,287; 5,256,526; 5,258,270; 5,272,051; 5,306,610; 5,326,682; 5,366,856; 5,378,596; 5,380,638; 5,382,502; 5,384,236; 5,397,691; 5,415,990; 5,434,034; 5,441,863; EP-A-0 246 616; EP-A-0 250 201; EP-A-0 271 323; EP-A-0 295 632; EP-A-0 307 927; EP-A-0 333 185; EP-A-0 378 898; EP-A-0 389 817; EP-A-0 487 111; EP-A-0 488 248; EP-A-0 539 034; EP-A-0 545 300; EP-A-0 556 700; EP-A-0 556 777; EP-A-0 556 858; EP-A-0 569 979; EP-A-0 608 133; EP-A-0 636 936; EP-A-0 651 286; EP-A-0 690 344; German OLS 4,026,903; German OLS 3,624,777 and German OLS 3,823,049. Typically such couplers are phenols, naphthols or pyrazoloazoles.

Couplers that form magenta dyes upon reaction with oxidized colour developing agent are described in such representative patents and publications as: "Farbkuppler-eine Literaturübersicht," published in Agfa Mitteilungen, Band III, pp. 126-156 (1961) as well as U.S. Pat. Nos. 2,311,082; 2,369,489; 2,343,701; 2,600,788; 2,908,573; 3,062,653; 3,152,896; 3,519,429; 3,758,309; 3,935,015; 4,540,654; 4,745,052; 4,762,775; 4,791,052; 4,812,576; 4,835,094; 4,840,877; 4,845,022; 4,853,319; 4,868,099; 4,865,960; 4,871,652; 4,876,182; 4,892,805; 4,900,657; 4,910,124; 4,914,013; 4,921,968; 4,929,540; 4,933,465; 4,942,116; 4,942,117; 4,942,118; 4,959,480; 4,968,594; 4,988,614; 4,992,361; 5,002,864; 5,021,325; 5,066,575; 5,068,171; 5,071,739; 5,100,772; 5,110,942; 5,116,990; 5,118,812; 5,134,059; 5,155,016; 5,183,728; 5,234,805; 5,235,058; 5,250,400; 5,254,446; 5,262,292; 5,300,407; 5,302,496; 5,336,593; 5,350,667; 5,395,968; 5,354,826; 5,358,829; 5,368,998; 5,378,587; 5,409,808; 5,411,841; 5,418,123; 5,424,179; EP-A-0 257 854; EP-A-0 284 240; EP-A-0 341 204; EP-A-0 347,235; EP-A-0 365,252; EP-A-0 422 595; EP-A-0 428 899; EP-A-0 428 902; EP-A-0 459 331; EP-A-0 467 327; EP-A-0 476 949; EP-A-0 487 081; EP-A-0 489 333; EP-A-0 512 304; EP-A-0 515 128; EP-A-0 534 703; EP-A-0 554 778; EP-A-0 558 145; EP-A-0 571 959; EP-A-0 583 832; EP-A-0 583 834; EP-A-0 584 793; EP-A-0 602 748; EP-A-0 602 749; EP-A-0 605 918; EP-A-0 622 672; EP-A-0 622 673; EP-A-0 629 912; EP-A-0 646 841; EP-A-0 656 561; EP-A-0 660 177; EP-A-0 686 872; WO 90/10253; WO 92/09010; WO 92/10788; WO 92/12464; WO 93/01523; WO 93/02392; WO 93/02393; WO 93/07534; UK Application 2,244,053; Japanese Application 03192-350; German OLS 3,624,103; German OLS 3,912,265 and German OLS 40 08 067. Typically such couplers are pyrazolones, pyrazoloazoles or pyrazolobenzimidazoles that form magenta dyes upon reaction with oxidized colour developing agents.

Couplers that form yellow dyes upon reaction with oxidized colour developing agent are described in such representative patents and publications as: "Farbkuppler-eine Literaturübersicht," published in Agfa Mitteilungen; Band III; pp. 112-126 (1961); as well as U.S. Pat. Nos. 2,298,443; 2,407,210; 2,875,057; 3,048,194; 3,265,506; 3,447,928; 4,022,620; 4,443,536; 4,758,501; 4,791,050; 4,824,771; 4,824,773; 4,855,222; 4,978,605; 4,992,360; 4,994,361; 5,021,333; 5,053,325; 5,066,574; 5,066,576; 5,100,773; 5,118,599; 5,143,823; 5,187,055; 5,190,848; 5,213,958; 5,215,877; 5,215,878; 5,217,857; 5,219,716; 5,238,803; 5,283,166; 5,294,531; 5,306,609; 5,328,818; 5,336,591; 5,338,654; 5,358,835; 5,358,838; 5,360,713; 5,362,617; 5,382,506; 5,389,504; 5,399,474; 5,405,737; 5,411,848; 5,427,898; EP-A-0 327 976; EP-A-0 296 793; EP-A-0 365 282; EP-A-0 379 309; EP-A-0 415 375; EP-A-0 437 818; EP-A-0 447 969; EP-A-0 542 463; EP-A-0 568 037; EP-A-0 568 196; EP-A-0 568 777; EP-A-0 570 006; EP-A-0 573 761; EP-A-0 608 956; EP-A-0 608 957 and EP-A-0 628 865. Such couplers are typically open chain ketomethylene compounds.

Couplers that form colourless products upon reaction with oxidized colour developing agent are described in such representative patents as: UK Patent No. 861,138; U.S. Pat. Nos. 3,632,345; 3,928,041; 3,958,993 and 3,961,959. Typically such couplers are cyclic carbonyl-containing compounds that form colourless products on reaction with an oxidized colour-developing agent.

Couplers that form black dyes upon reaction with oxidized colour developing agent are described in such representative patents as U.S. Pat. Nos. 1,939,231; 2,181,944; 2,333,106 and 4,126,461; German OLS No. 2,644,194 and German OLS No. 2,650,764. Typically, such couplers are resorcinols or m-aminophenols that form black or neutral products on reaction with oxidized colour-developing agent.

In addition to the foregoing, so-called "universal" or "washout" couplers may be employed. These couplers do not contribute to image dye-formation. Thus, for example, a naphthol having an unsubstituted carbamoyl or one substituted with a low molecular weight substituent at the 2- or 3-position may be employed. Couplers of this type are described, for example, in U.S. Pat. Nos. 5,026,628, 5,151,343 and 5,234,800.

It may be useful to use a combination of couplers any of which may contain known ballasts or coupling-off groups such as those described in U.S. Pat. Nos. 4,301,235; 4,853,319 and U.S. Pat. No. 4,351,897. The coupler may contain solubilizing groups such as described in U.S. Pat. No. 4,482,629. The coupler may also be used in association with "wrong" coloured couplers (e.g. to adjust levels of interlayer correction) and, in colour negative applications, with masking couplers such as those described in EP-A-0 213,490; Japanese Published Application 58-172,647; U.S. Pat. Nos. 2,983,608; 4,070,191 and 4,273,861; German Applications DE 2,706,117 and DE 2,643,965; UK Patent No. 1,530,272; and Japanese Application 58-113935. The masking couplers may be shifted or blocked, if desired.

The materials for use in the invention may be used in association with materials that release PUGs that accelerate or otherwise modify the processing steps e.g. of bleaching or fixing to improve the quality of the image. Bleach accelerator-releasing couplers, such as those described in EP-A-0 193,389; EP-A-0 301,477 and in U.S. Pat. Nos. 4,163,669, 4,865,956 and 4,923,784, may be useful. Also contemplated is use of the compositions in association with nucleating agents, development accelerators or their precursors (UK Patent Nos. 2,097,140 and 2,131,188); electron transfer agents (U.S. Pat. Nos. 4,859,578 and 4,912,025); antifogging and anticolour-

mixing agents such as derivatives of hydroquinones, aminophenols, amines, gallic acid; catechol; ascorbic acid; hydrazides; sulfonamidophenols and noncolour-forming couplers.

The materials for use in the invention may also be used in combination with filter dye layers comprising yellow, cyan, and/or magenta filter dyes, either as oil-in-water dispersions, latex dispersions or as solid particle dispersions. Additionally, they may be used with "smearing" couplers (e.g. as described in U.S. Pat. Nos. 4,366,237, 4,420,556, 4,543,323 and EP-A-0 96,570). (Also, the compositions may be blocked or coated in protected form as described, for example, in Japanese Application 61/258,249 or U.S. Pat. No. 5,019,492.

The materials for use in the invention may further be used in combination with image-modifying compounds that release PUGs such as "Developer Inhibitor-Releasing" compounds (DIRs). DIRs useful in conjunction with the compositions useful in the invention are known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,411; 346,899; 362,870; 365,252; 365,346; 373,382; 376,212; 377,463; 378,236; 384,670; 396,486; 401,612; 401,613.

Such compounds are also disclosed in "Developer-Inhibitor-Releasing (DIR) Couplers for Colour Photography," C. R. Barr, J. R. Thirtle and P. W. Vittum in *Photographic Science and Engineering*, Vol. 13, p. 174 (1969), incorporated herein by reference. Generally, the developer inhibitor-releasing (DIR) couplers include a coupler moiety and an inhibitor coupling-off moiety (IN). The inhibitor-releasing couplers may be of the time-delayed type (DIAR couplers) that also include a timing moiety or chemical switch that produces a delayed release of inhibitor. Examples of typical inhibitor moieties are: oxazoles, thiazoles, diazoles, triazoles, oxadiazoles, thiadiazoles, oxathiazoles, thiatriazoles, benzotriazoles, tetrazoles, benzimidazoles, indazoles, isoindazoles, mercapto-tetrazoles, selenotetrazoles, mercaptobenzothiazoles, selenobenzothiazoles, mercaptobenzoxazoles, selenobenzoxazoles, mercaptobenzimidazoles, selenobenzimidazoles, benzodiazoles, mercaptodoxazoles, mercaptothiadiazoles, mercaptothiazoles, mercaptotriazoles, mercaptooxadiazoles, mercaptodiazoles, mercaptooxathiazoles, tellurotetrazoles or benzisodiazoles. In a preferred embodiment, the inhibitor moiety or group is selected from the following formulae:





wherein  $R_I$  is selected from the group comprising straight and branched alkyl groups of from 1 to about 8 carbon atoms, benzyl, phenyl, and alkoxy groups and such groups containing none, one or more than one such substituent;  $R_{II}$  is selected from  $R_I$  and  $-SR_I$ ;  $R_{III}$  is a straight or branched alkyl group of from 1 to about 5 carbon atoms and  $m$  is from 1 to 3; and  $R_{IV}$  is selected from the group comprising hydrogen, halogen, and alkoxy, phenyl and carboxamido groups,  $-CO-OR_V$  and  $-NHCOOR_V$  wherein  $R_V$  is selected from substituted and unsubstituted alkyl and aryl groups.

Although it is typical that the coupler moiety included in the developer inhibitor-releasing coupler forms an image dye corresponding to the layer in which it is located, it may also form a different colour as one associated with a different film layer. It may also be useful that the coupler moiety included in the developer inhibitor-releasing coupler forms colourless products and/or products that wash out of the photographic material during processing (so-called "universal" couplers).

A compound such as a coupler may release a PUG directly upon reaction of the compound during processing, or indirectly through a timing or linking group. A timing group produces the time-delayed release of the PUG, such groups using an intramolecular nucleophilic substitution reaction (U.S. Pat. No. 4,248,962); groups utilizing an electron transfer reaction along a conjugated system (U.S. Pat. Nos. 4,409,323, 4,421,845 and 4,861,701, Japanese Applications 57-188035; 58-98728; 58-209736; 58-209738); groups that function as a coupler or reducing agent after the coupler reaction (U.S. Pat. Nos. 4,438,193 and 4,618,571) and groups that combine the features described above. It is typical that the timing group is of one of the formulae:



wherein IN is the inhibitor moiety, Z is selected from the group comprising nitro, cyano, alkyl- or aryl-sulfonyl; alkyl- or aryl-sulfamoyl and allyl- or aryl-sulfonamido groups;  $n$  is 0 or 1; and  $R_{VI}$  is selected from the group comprising substituted and unsubstituted alkyl and phenyl groups. The oxygen atom of each timing group is bonded to the coupling-off position of the respective coupler moiety of the DIAR.

The timing or linking groups may also function by electron transfer down an unconjugated chain. Linking groups are

known in the art under various names. Often they have been referred to as groups capable of utilizing a hemiacetal or iminoketal cleavage reaction or as groups capable of utilizing a cleavage reaction due to ester hydrolysis such as U.S. Pat. No. 4,546,073. This electron transfer down an unconjugated chain typically results in a relatively fast decomposition and the production of carbon dioxide, formaldehyde, or other low molecular weight by-products. The groups are exemplified in 10 EP-A-0 464,612, EP-A-0 523,451, U.S. Pat. No. 4,146,396 and Japanese Kokais 60-249148 and 60-249149.

Suitable developer inhibitor-releasing couplers that may be included in photographic light-sensitive emulsion layer include, but are not limited to, the following:



**35**

-continued

**36**

-continued



D9



D10



D11



D12

A light-sensitized silver halide emulsion layer is a sublayer of the photographic film that contains light-sensitized silver halide crystals incorporated as an emulsion in the sublayer, utilizing emulsifying agents such as, but not limited to, gelatin. Silver halide is light-sensitized by the use of sensitizing dyes that are adsorbed to the silver halide crystals and that capture scene light and initiate formation of the scene latent image silver.

Especially useful in this invention are tabular grain silver halide emulsions. Tabular grains are those having two parallel major crystal faces and having an aspect ratio of at least 2. The term "aspect ratio" is the ratio of the equivalent circular diameter (ECD) of a grain major face divided by its thickness (t). The major faces of the tabular grains can lie in either {111} or {100} crystal planes. Specifically contemplated tabular grain emulsions are those in which greater than 50% of the total projected area of the emulsion grains are accounted for by tabular grains having a thickness of less than 0.3  $\mu\text{m}$  (0.5  $\mu\text{m}$  for blue sensitive emulsion) and an average tabularity (T) of greater than 25 (preferably greater than 100), where the term "tabularity" is employed in its art recognized usage as

$$T = ECD/t^2$$

wherein ECD is the average equivalent circular diameter of the tabular grains in micrometers and t is the average thickness in micrometers of the tabular grains.

The average useful ECD of photographic emulsions can range up to about 10  $\mu\text{m}$ , although in practice emulsion ECDs seldom exceed about 4  $\mu\text{m}$ . Since both photographic speed and granularity increase with increasing ECDs, it is generally preferred to employ the smallest tabular grain ECDs compatible with achieving aim speed requirements.

Emulsion tabularity increases markedly with reductions in tabular grain thickness. It is generally preferred that aim tabular grain projected areas be satisfied by thin (t less than 0.2  $\mu\text{m}$ ) tabular grains. To achieve the lowest levels of granularity it is preferred that aim tabular grain projected areas be satisfied with ultrathin (t less than 0.07  $\mu\text{m}$ ) tabular grains. Tabular grain thicknesses typically range down to about 0.02  $\mu\text{m}$ . However, still lower tabular grain thicknesses are contemplated. For example, Daubendiek et al. U.S. Pat. No. 4,672,027 reports a 3-mol % iodide tabular grain silver bromoiodide emulsion having a grain thickness of 0.017  $\mu\text{m}$ . Ultrathin tabular grain high chloride emulsions are disclosed by Maskasky in U.S. Pat. No. 5,217,858.

As noted above tabular grains of less than the specified thickness account for at least 50% of the total grain projected area of the emulsion. To maximize the advantages of high tabularity it is generally preferred that tabular grains satisfying the stated thickness criterion account for the highest conveniently attainable percentage of the total grain projected area of the emulsion. For example, in preferred emulsions, tabular grains satisfying the stated thickness criteria above account for at least 70% of the total grain projected area. In the highest performance tabular grain emulsions, tabular grains satisfying the thickness criteria above account for at least 90% of total grain projected area.

Suitable tabular grain emulsions can be selected from among a variety of conventional teachings, such as those of the following Research Disclosure, Item 22534, January 1983, published by Kenneth Mason Publications, Ltd., Emsworth, Hampshire PO10 7DD, England; U.S. Pat. Nos. 4,439,520; 4,414,310; 4,433,048; 4,643,966; 4,647,528; 4,665,012; 4,672,027; 4,678,745; 4,693,964; 4,713,320; 4,722,886; 4,755,456; 4,775,617; 4,797,354; 4,801,522;

4,806,461; 4,835,095; 4,853,322; 4,914,014; 4,962,015; 4,985,350; 5,061,069 and 5,061,616. Tabular grain emulsions comprising predominantly silver chloride are useful and are described, for example, in U.S. Pat. Nos. 5,310,635; 5,320,938 and 5,356,764.

In their most widely used form tabular grain emulsions are high bromide {111} tabular grain emulsions. Such emulsions are illustrated by Kofron et al U.S. Pat. No. 4,439,520, Wilgus et al U.S. Pat. No. 4,434,226, Solberg et al, U.S. Pat. No. 10 4,433,048, Maskasky U.S. Pat. Nos. 4,435,501, 4,463,087 and 4,173,320, Daubendiek et al U.S. Pat. Nos. 4,414,310 and 4,914,014, Sowinski et al U.S. Pat. No. 4,656,122, Pigglin et al U.S. Pat. Nos. 5,061,616 and 5,061,609, Tsaur et al U.S. Pat. Nos. 5,147,771, 5,147,772, 5,147,773, 5,171,659 and 5,252, 15 453, Black et al U.S. Pat. Nos. 5,219,720 and 5,334,495, Delton U.S. Pat. Nos. 5,310,644, 5,372,927 and 5,460,934, Wen U.S. Pat. No. 5,470,698, Fenton et al U.S. Pat. No. 5,476,760, Eshelman et al U.S. Pat. Nos. 5,612,175 and 5,614,359, and Irving et al U.S. Pat. No. 5,667,954.

20 Ultrathin high bromide {111} tabular grain emulsions are illustrated by Daubendiek et al U.S. Pat. Nos. 4,672,027, 4,693,964, 5,494,789, 5,503,971 and 5,576,168, Antoniades et al U.S. Pat. No. 5,250,403, Olm et al U.S. Pat. No. 5,503, 25 970, Deaton et al U.S. Pat. No. 5,582,965 and Maskasky U.S. Pat. No. 5,667,955.

High bromide {100} tabular grain emulsions are illustrated by Mignot U.S. Pat. Nos. 4,386,156 and 5,386,156.

High chloride {111} tabular grain emulsions are illustrated by Wey U.S. Pat. No. 4,399,215, Wey et al U.S. Pat. No. 30 4,414,306, Maskasky U.S. Pat. Nos. 4,400,463, 4,713,323, 5,061,617, 5,178,997, 5,183,732, 5,185,239, 5,399,478 and 5,411,852, and Maskasky et al U.S. Pat. Nos. 5,176,992 and 5,178,998. Ultrathin high chloride {111} tabular grain emulsions are illustrated by Maskasky U.S. Pat. Nos. 5,271,858 and 5,389,509. High chloride {100} tabular grain emulsions are illustrated by Maskasky U.S. Pat. Nos. 5,264,337, 5,292, 632, 5,275,930 and 5,399,477, House et al U.S. Pat. No. 5,320,938, Brust et al U.S. Pat. No. 5,314,798, Szajewski et al U.S. Pat. No. 5,356,764, Chang et al U.S. Pat. Nos. 5,413,904 and 5,663,041, Oyamada U.S. Pat. No. 5,593,821, Yamashita et al U.S. Pat. Nos. 5,641,620 and 5,652,088, Saitou et al U.S. Pat. No. 5,652,089, and Oyamada et al U.S. Pat. No. 5,665, 45 530. Ultrathin high chloride {100} tabular grain emulsions can be prepared by nucleation in the presence of iodide, following the teaching of House et al and Chang et al, cited above.

The emulsions can be surface-sensitive emulsions, i.e., emulsions that form latent images primarily on the surfaces of the silver halide grains, or the emulsions can form internal latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is conducted with uniform light exposure or in the presence of a nucleating agent. Tabular grain emulsions of the latter type are illustrated by Evans et al in U.S. Pat. No. 4,504,570.

60 Photographic elements can be exposed to actinic radiation, typically in the visible region of the spectrum, to form a latent image and can then be processed to form a visible dye image. Processing to form a visible dye image includes the step of contacting the element with a colour developing agent to reduce developable silver halide and oxidize the colour developing agent. Oxidized colour developing agent in turn reacts with the coupler to yield a dye.

39

With negative-working silver halide, the processing step described above provides a negative image. One type of such element, referred to as a colour negative film, is designed for image capture. Speed (the sensitivity of the element to low light conditions) is usually critical to obtaining sufficient image in such elements. Such elements are typically silver bromoiodide emulsions and may be processed, for example, in known colour negative processes such as the Kodak C-41™ process as described in The British Journal of Photography Annual of 1988, pages 191-198. If a colour negative film element is to be subsequently employed to generate a viewable projection print as for a motion picture, a process such as the Kodak ECN-2™ process described in the H-24 Manual available from Eastman Kodak Co. may be employed to provide the colour negative image on a transparent support. Colour negative development times are typically 3 min 15 s. The photographic element of the invention can be incorporated into exposure structures intended for repeated use or exposure structures intended for limited use, variously referred to by names such as "single use cameras", "lens with film", or "photosensitive material package units".

A reversal element is capable of forming a positive image without optical printing. To provide a positive (or reversal) image, the colour development step is preceded by development with a nonchromogenic developing agent to develop exposed silver halide, but not form dye and followed by uniformly fogging the element to render unexposed silver halide developable. Such reversal emulsions are typically sold with instructions to process using a colour reversal process such as the Kodak E-6™ process. Alternatively, a direct positive emulsion can be employed to obtain a positive image.

The above emulsions are typically sold with instructions to process using the appropriate method such as the mentioned colour negative (Kodak C-41™) or reversal (Kodak E-6™) process.

Preferred colour developing agents are p-phenylenediamines such as: 4-amino-N,N-diethylaniline hydrochloride, 4-amino-3-methyl-N,N-diethylaniline hydrochloride, 4-amino-3-methyl-N-ethyl-N-(2-methanesulfonamidoethyl)aniline sesquisulfate hydrate,

4-amino-3-methyl-N-ethyl-N-(2-hydroxyethyl)aniline sulfate,

4-amino-3-(2-methanesulfonamidoethyl)-N,N-diethylaniline hydrochloride, and

4-amino-N-ethyl-N-(2-methoxyethyl)-m-toluidine di-p-toluene sulfonic acid.

Of the above, developers based on 4-amino-3-methyl-N-ethyl-N-(2-hydroxyethyl)aniline and 4-amino-3-methyl-N-ethyl-N-(2-methane-sulfonamidoethyl)aniline are especially preferred. Moreover, because the compounds useful in the invention give increased light sensitivity, they are especially useful in processes that have shortened development times. In particular, the film elements of the invention can be processed with development times of less than 3.25 min or even less than 3 min or in extreme cases, even less than 120 s.

Development is usually followed by the conventional steps of bleaching, fixing, or bleach-fixing to remove silver or silver halide, washing and drying.

The invention will now be described with reference to the following examples which are no way to be interpreted as limiting the scope thereof.

40

## EXAMPLES

## Synthesis of Compounds of Formula (I)

## Example 1

## Synthesis of SGA1

## a) 2-(3-Pentadecylphenoxy)butanoyl chloride

2-(3-Pentadecylphenoxy)butanoic acid (4.18 g, 0.01 mol) (CAS Registry Number 14230-52-5) and thionyl chloride (30 ml) were heated under reflux on a steam-bath for 1 h. The resulting yellow solution was allowed to cool before being distilled under reduced pressure to leave a yellow oil. The oil was dissolved in dichloromethane (50 ml) and the solution was distilled under reduced pressure to remove volatiles. The residual 2-(3-pentadecylphenoxy)butanoyl chloride was used without further purification.

## b) SGA1

A solution of 2-(3-pentadecylphenoxy)butanoyl chloride (0.01 mol) in tetrahydrofuran (30 ml) was added dropwise to a dark brown suspension of 2-aminoimidazole sulfate (1.5 g, 0.011 mol, Aldrich) in pyridine (30 ml) at room temperature and the mixture was stirred for 18 h. The brown suspension was poured into stirred water (700 ml) which contained 10M hydrochloric acid (100 ml) and the resulting oil was extracted into dichloromethane (100 ml). The extract was washed with water before being dried over magnesium sulfate and then the solvent was distilled off under reduced pressure from the dried solution. The orange residue was recrystallised from a mixture of acetonitrile, ethyl acetate and methanol to give a pink solid. The solid was recrystallised from methanol to give SGA1 as a pale pink solid, 1.23 g (25%).

## Example 2

## The Synthesis of SGA2

## a) 2-(2,4-Di-t-pentylphenoxy)ethanoyl chloride

2-(2,4-Di-t-pentylphenoxy)ethanoic acid (12.0 g, 0.041 mol) (CAS Registry Number 13402-96-5) and thionyl chloride (60 ml) were heated under reflux on a steam-bath for 1.5 h. The resulting yellow solution was allowed to cool before being distilled under reduced pressure to remove volatiles. The residue was dissolved in 60-80 petroleum-ether (200 ml) and the solution was distilled under reduced pressure to remove any remaining traces of volatiles, leaving 2-(2,4-di-t-pentyl-phenoxy)ethanoyl chloride as a red oil which was used without further purification.

## b) SGA2

A solution of 2-(2,4-di-t-pentylphenoxy)ethanoyl chloride (0.041 mol) in tetrahydrofuran (60 ml) was added dropwise to a stirred solution of 2-amino-4,5-dicyanoimidazole (5.47 g, 0.041 mol, Aldrich) in pyridine (60 ml) at ambient temperature and the resulting brown suspension was stirred for 20 h. The reaction mixture was then poured into a mixture of water (1250 ml) and 10M hydrochloric acid (200 ml) and the resulting solid was filtered off and recrystallized from acetonitrile/tetrahydrofuran to give SGA2 as a dull pink solid, 4.42 g (26%).

41

Example 3

## The Synthesis of SGA21

A yellow suspension of benzil (19.69 g, 0.09 mol) (CAS Registry Number 134-81-6) 2-furaldehyde (10 g, 0.1 mol) (CAS Registry Number 98-01-1) and ammonium acetate (20 g, 0.26 mol) in acetic acid (100 ml) was heated at 12° C. for 18 h. After this time the dark brown solution was poured into water (500 ml) and the resulting black solid filtered off and stirred over acetonitrile for 18 h. Filtration gave the product, SGA21, as a dark green solid (19.98 g, 67%).

## Photographic Examples

Multilayer films demonstrating the principles of this invention were produced by coating the following layers on a cellulose triacetate film support (coverage are in g/m<sup>2</sup>, emulsion sizes as determined by the disc centrifuge method and are reported in diameter×thickness in micrometers). Surfactants, coating aids, emulsion addenda (including 4-hydroxy-6-methyl-1,3,3a,7-tetra-azaindene), sequestrants, thickeners, lubricants, matte and tinting dyes were added to the appropriate layers as is common in the art. Formulae for the identified compounds are provided at the end of these examples.

Layer 1 (Antihalation layer): gelatin at 1.08, colloidal gray silver at 0.150; ILS-1 at 0.097; DYE-1 at 0.029; DYE-2 at 0.065; DYE-3 at 0.021; CH-1 at 0.025 and UV-1 at 0.075.

Layer 2 (Slow cyan layer): a blend of two red-sensitized (all with a mixture of RSD-1 and RSD-2) tabular silver iodobromide emulsions: (i) 0.81×0.11 µm, 4.5 mol % I at 0.400, (ii) 0.62×0.111 µm, 4.1 mol % iodide at 0.175; cyan dye-forming couplers C-1 at 0.248 and C-2 at 0.236; bleach-accelerator releasing coupler B-1 at 0.086; image-modifier DIR-1 at 0.032; OxDs-1 at 0.010 and gelatin at 1.08.

Layer 3 (Mid cyan layer): a red-sensitized (with a mixture of RSD-1 and RSD-2) iodobromide tabular emulsion (1.44×0.13 µm, 3.7 mol % I) at 0.572; C-1 at 0.265; C-2 at 0.103; B-1 at 0.011; DIR-2 at 0.043; masking coupler MC-1 at 0.022 and gelatin at 1.08.

Layer 4 (Fast cyan layer): a red-sensitized (with a mixture of RSD-1, RSD-2 and RSD-3) iodobromide tabular emulsion (2.41×0.13 µm, 3.7 mol % I) at 1.286; C-1 at 0.163; DIR-2 at 0.054; B-1 at 0.008 and gelatin at 1.08.

Layer 5 (Ultra-fast cyan layer): a red-sensitized (with a mixture of RSD-1, RSD-2 and RSD-3) iodobromide tabular emulsion (3.87×0.13 µm, 3.7 mol % I) at 1.180; C-2 at 0.175; DIR-3 at 0.060; DIR-4 at 0.001 and gelatin at 1.08.

Layer 6 (Interlayer): ILS-1 at 0.075 and gelatin at 1.08.

Layer 7 (Slow magenta layer): a blend of two green-sensitized (both with a mixture of GSD-1 and GSD-2) silver iodobromide tabular emulsions:

(i) 1.17×0.12 µm, 4.5 mol % iodide at 0.156 and (ii) 0.62×0.111 µm, 2.6 mol % iodide at 0.573; magenta dye-forming coupler M-1 at 0.300; MC-2 at 0.090, DIR-5 at 0.032, ILS-1 at 0.011 and gelatin at 1.400.

Layer 8 (Mid magenta layer): a blend of two green-sensitized (both with a mixture of GSD-1 and GSD-2) silver iodobromide tabular emulsions:

(i) 2.46×0.13 µm, 3.7 mol % iodide at 0.534 and (ii) 1.45×0.13 µm, 3.7 mol % iodide at 0.370; M-1 at 0.089; MC-2 at 0.086; DIR-5 at 0.025, ILS-1 at 0.012 and gelatin at 1.438.

42

Layer 9 (Fast magenta layer): two parts mixed together at a 1:1 ratio just prior to coating; Part A (dispersion melt): M-1 at 0.104; DIR-5 at 0.011; ILS-1 at 0.014 and gelatin at 0.420 and Part B (emulsion melt): a green-sensitized (with a mixture of GSD-1 and GSD-2) silver iodobromide tabular emulsion (2.90×0.13 µm, 3.7 mol % iodide) at 1.240; MC-2 at 0.021; DIR-6 at 0.003 and gelatin at 1.076.

Layer 10 (Interlayer): ILS-1 at 0.182 and gelatin at 0.700.

Layer 11 (Slow yellow layer): a blend of three blue-sensitized (all with BSD-1 and BSD-2) tabular silver iodobromide emulsions (i) 2.41×0.1 µm, 2.0 mol % I at 0.402, (ii) 1.02×0.137 µm, 2.0 mol % I at 0.136, (iii) 0.62×0.111 µm, 2.6 mol % I at 0.505; yellow dye-forming coupler Y-1 at 0.850; DIR-1 at 0.022; DIR-7 at 0.038; B-1 at 0.009 and gelatin at 1.90.

Layer 12 (Fast yellow layer): a blue-sensitized (with BSD-1 and BSD-2) tabular silver iodobromide emulsion, 3.72×0.131 µm, 3.7 mol % I at 0.070 and a blue-sensitized (with BSD-1) 3-D silver iodobromide emulsion, 1.21 µm diameter), 9.7 mol % I at 1.055; Y-1 at 0.312; DIR-7 at 0.065; B-1 at 0.011, stabiliser S-1 at 0.008 and gelatin at 1.280.

Layer 13 (UV Filter Layer): silver bromide Lippman emulsion at 0.215; UV-1 and UV-2 both at 0.108 and gelatin at 0.700.

Layer 14 (Protective overcoat): gelatin at 0.888 and bis(vinylsulfonyl)methane hardener at 1.75% of total gelatin weight.

All comparative and imidazole compounds were dispersed in twice their own weight in N,N-dibutyl lauramide unless otherwise noted. All parts containing the comparative or imidazole compounds were stirred at 40C for at least 1 h before coating. Comparative samples of the invention had the test compound added at 0.0806 mmol/m<sup>2</sup> to Part A of Layer 9.

Formulae for materials used in the above formats are as follows:—

ILS-1:



DYE-1:



**43**DYE-2:  
-continued

DYE-3:



CH-1:



UV-1:



C-1:

**44**

-continued

C-2:



B-1:



DIR-1:



OxDS-1:



**45**DIR-2:  
-continued

MC-1:



DIR-3:



DIR-4:

**46**

-continued

M-1:



MC-2:



DIR-5:



**47**DIR-6:  
-continued

Y-1:

DIR-7:



S-1:

UV-2:

**48**BSD-1:  
-continued

5



BSD-2:



GSD-1:



50 GSD-2:



RSD-1:

-continued



RSD-2:



RSD-3:



Comparative compounds

CC1



CC2



CC3



To determine speed these multilayer coatings were given a stepped neutral exposure and processed in the KODAK FLEXICOLOUR™ (C-41) process as described in *British Journal of Photography Annual*, 1988, pp 196-198. Speed or light sensitivity (given in terms of fraction of a stop) is inversely related to the exposure required to produce a specified film density ( $D_s$ ) in the toe of a sensitometric DlogE curve of  $0.2 \times$  gradient ( $\gamma$ ) at that density above  $D_{min}$ , i.e.

$$D_s = 0.2\gamma + D_{min}$$

10

The speed corresponds to the exposure which can be computed from  $D_s$  from the DlogE curve. A larger, more positive number means increased speed: a negative number means a loss in speed. Granularity of the green layer in a neutral exposure was determined by the RMS method (see *The Theory of the Photographic Process*, 4<sup>th</sup> Edition, T. H. James, pp 625-628) using a 48 micrometer aperture at the density 1.2 log exposure units from the speed point defined above.

Photographic data which illustrate the imidazole compounds are given in the tables below, wherein  $\Delta$  Speed is the difference in speed between the check, the comparative compounds and the imidazole compounds.

TABLE 1

| Speed/Grain Addendum | $\Delta$ Speed (stops) | C/I |
|----------------------|------------------------|-----|
| SGA1                 | 0.07                   | I   |
| CC1                  | -0.23                  | C   |

It will be seen that comparative benzimidazole compound CC1, having no  $-\text{NH}$  group attached to the carbon between the imidazole nitrogen atoms, shows a speed loss whereas the imidazole SGA1 has a speed gain of 0.07 stop.

TABLE 2

| Speed/Grain Addendum | $\Delta$ Speed (stops) | Granularity $\times 10^3$ | C/I |
|----------------------|------------------------|---------------------------|-----|
| Check                |                        | 21                        | C   |
| SGA2                 | 0.13                   | 19                        | I   |
| SGA21                | 0.07                   | 19                        | I   |
| CC2                  | 0                      | 19                        | C   |
| CC3                  | 0                      | 19                        | C   |

The data in the table show that the photographic speed of an element which contains a 'speed/grain' addendum is increased compared to the photographic element without the 'speed/grain' addendum.

For example, comparative compound CC2, with no  $-\text{NH}$  group either on the ring or as an exocyclic substituent directly attached to the imidazole ring, does not show a speed gain, whereas SGA21 of similar structure but with a ring  $-\text{NH}$  group shows a speed gain of 0.07 stop. It can be seen also that

SGA2 with three electron-withdrawing groups (carbonyl and two cyan groups) has an enhanced speed gain of 0.13 stop compared with SGA21, which has only one electron-withdrawing group (a furanyl group). Comparative compound CC3 which has a ring  $-\text{NH}$  and is fused to a phenanthrene ring, and expressly excluded in this invention, shows no speed gain whilst SGA21, which also has a ring  $-\text{NH}$ , but with separate phenyl substituents on the imidazole ring, exhibits a speed gain of 0.07 stop.

The entire contents of the patent and publications referred to in this specification are incorporated herein by reference.

The invention has been described in detail with particular reference to preferred embodiments thereof but it will be

## 51

understood that variations and modifications can be effected within the spirit and scope of the invention.

The invention claimed is:

1. A colour photographic element comprising at least one light-sensitive silver halide emulsion layer or a non silver-containing light-insensitive layer, in which at least one of these layers contains a colourless imidazole compound of formula (I) that undergoes less than 10% chemical or redox reaction directly with oxidized developer and which enables the photographic speed of the element to be increased by at least 0.03 stop without increasing granularity, compared to the same element without the compound, wherein the compound of formula (I) has the structure:—



wherein

X is H or a substituent;

Z represents the atoms necessary to complete an unsubstituted or substituted imidazole ring, which may form part of a fused unsubstituted or substituted ring system containing no further ring heteroatoms;

wherein there is present at least one —NH group either in the imidazole ring or directly attached to the imidazole ring as part of X;

provided that

(a) when Z represents the atoms necessary to complete an unsubstituted or substituted benzimidazole ring, an —NH group is directly attached to the imidazole ring as part of X, and X is located between the imidazole nitrogen atoms;

(b) when the —NH group is located in the ring adjacent to the carbon atom bearing X, and X is located between the imidazole nitrogen atoms, the imidazole ring is not fused to a phenanthrene ring.

2. A colour photographic element as claimed in claim 1 wherein the compound of formula (I) undergoes less than 5% chemical or redox reaction directly with oxidised developer.

3. A colour photographic element as claimed in either of the preceding claims wherein the compound of formula (I) is contained in the most light-sensitive layer of two or more light-sensitive layers having the same spectral sensitivity.

4. A colour photographic element as claimed in any one of the preceding claims wherein the compound of formula (I) is located in the green record wherein the maximum spectral sensitivity to light is from 500 to 600 nm.

5. A colour photographic element as claimed in any one of the preceding claims wherein the silver halide comprises silver iodobromide.

6. A colour photographic element as claimed in any one of the preceding claims wherein the compound of formula (I) enables the photographic speed of the element to be increased by at least 0.10 stop without increasing granularity, compared to the same element without the compound.

7. A colour photographic element as claimed in any one of the preceding claims wherein the compound of formula (I) has one or more electron-withdrawing groups attached to the imidazole ring, a ring fused thereto or as part of substituent X.

8. A colour photographic element as claimed in any one of the preceding claims wherein when there is an —NH group as part of the imidazole ring X is selected from a cyano or an unsubstituted or substituted alkyl, aryl, alkyl- or aryl-sulfonyl, alkyl- or aryl-carbonyl, alkyl- or aryl-carbonyl, heterocycl or a group NRQR<sup>1</sup>, wherein R is hydrogen or an alkyl group, R<sup>1</sup> is a substituent and Q is a carbonyl, sulfonyl or aryl group.

## 52

9. A colour photographic element as claimed in any one of the preceding claims wherein the compound has the formula (II)



10. wherein

NHQ is selected from the class consisting of amido, arylamino, ureido, carbamato or sulfonamido;

R<sup>1</sup> is a substituent; and

Z represents the atoms necessary to complete an unsubstituted or substituted imidazole ring, which may form part of a fused unsubstituted or substituted ring system containing no further ring heteroatoms; provided that when Z represents the atoms necessary to complete an unsubstituted or substituted benzimidazole ring, NHQR<sup>1</sup> is located between the two imidazole nitrogen atoms.

10. A colour photographic element as claimed in claim 9 wherein Q is or contains an electron-withdrawing group.

11. A colour photographic element as claimed in either of claims 9 and 10 wherein Q is or contains a carbonyl or a sulfonyl group.

12. A colour photographic element as claimed in claim 11 wherein, when Q is or contains a carbonyl group, the ring or ring system represented by Z contains one or more electron-withdrawing groups.

13. A colour photographic element as claimed in claim 11 wherein, when Q is or contains a sulfonyl group, the ring or ring system represented by Z is unsubstituted or contains one or more electron-withdrawing or electron-donating groups.

14. A colour photographic element as claimed in claim 9 wherein, when Q is an aryl group, the ring or ring system represented by Z contains one or more electron-withdrawing groups.

15. A colour photographic element as claimed in any one of claims 9 to 14 wherein the compound has the structure (III):—



50. wherein

R<sup>1</sup>, R<sup>2</sup>, R<sup>3</sup> and R<sup>4</sup> are independently selected substituents or R<sup>3</sup> and R<sup>4</sup> may join to form a fused ring not containing any ring heteroatoms;

55. NHQ is selected from the class consisting of an amido, ureido arylamino, carbamato or sulfonamido group.

16. A colour photographic element as claimed in claim 15 wherein R<sup>1</sup> is selected from hydrogen and an unsubstituted or substituted alkyl, aryl, alkoxy, aryloxy, or alkyl- or arylamino group.

17. A colour photographic element as claimed in either of claims 15 and 16 wherein, when Q is a carbonyl group, R<sup>1</sup> is an alkyl group which is unsubstituted or substituted with an unsubstituted or substituted aryloxy group.

60. 18. A colour photographic element as claimed in either of claims 15 and 16 wherein, when Q is a sulfonyl group, R<sup>1</sup> is a substituted aryl group.

53

19. A colour photographic element as claimed in either of claims **15** and **16** wherein, when Q is an aryl group, R<sup>1</sup> is an alkoxy group.

20. A colour photographic element as claimed in any one of claims **9** to **19** wherein R<sup>2</sup> is hydrogen or an unsubstituted or substituted alkyl group. 5

21. A colour photographic element as claimed in any one of claims **9** to **20** wherein at least one of R<sup>3</sup> and R<sup>4</sup> is hydrogen or a group which is independently selected from cyan, formyl, keto, carboxylic acid, mercapto and unsubstituted or substituted alkyl, aryl, alkoxy, aryloxy, alkoxy- or aryloxy-carbonyl, alkyl- or aryl-carbonyl, alkyl- or aryl-thio, alkyl- or aryl-sulfonyl, alkyl- or aryl-sulfonyl, alkyl- or aryl-carbamoyl and alkyl- or aryl-carbonamido, or R<sup>3</sup> and R<sup>4</sup> may join to form a fused ring. 10

22. A colour photographic element as claimed in any one of the preceding claims wherein the compound of formula (I) is selected from

SGA1



SGA2



and

54

-continued

SGA2I



15 23. A colour photographic element as claimed in any one of the preceding claims wherein when the compound is present in a sensitized layer the ratio of compound to silver is at least 0.1 mmol compound per mol silver halide.

20 24. A colour photographic element as claimed in any one of claims **1** to **22** wherein when the compound is present in a non-silver-containing layer, the laydown of the compound is at least  $3 \times 10^{-5}$  mol/m<sup>2</sup>.

25 25. A multi-colour photographic element comprising a support bearing yellow, magenta and cyan image-dye-forming units comprising at least one blue-, green- or red-sensitive silver halide emulsion layer having associated therewith at least one yellow, magenta or cyan dye-forming coupler respectively, wherein the element is as claimed in any one of the preceding claims.

30 26. A process of forming an image in a photographic element as hereinbefore defined after the element has been imagewise exposed to light, comprising contacting the element as claimed in any one of claims **1** to **25** with a colour developing agent.

\* \* \* \* \*